

# United States Patent

[19]

Yaffe

[11] 3,887,631

[45] June 3, 1975

[54] OXIDATIVE DEHYDROGENATION OF HYDROCARBONS

[75] Inventor: Roberta Yaffe, Fishkill, N.Y.

[73] Assignee: Texaco Inc., New York, N.Y.

[22] Filed: May 14, 1973

[21] Appl. No.: 359,953

[52] U.S. Cl. .... 260/680 E; 252/432; 260/683.3

[51] Int. Cl. .... C07c 5/18

[58] Field of Search ..... 260/680 E

## [56] References Cited

### UNITED STATES PATENTS

|           |         |                      |           |
|-----------|---------|----------------------|-----------|
| 3,159,688 | 12/1964 | Jennings et al. .... | 260/680 E |
| 3,320,330 | 5/1967  | Callahan et al. .... | 260/680 E |
| 3,380,931 | 4/1968  | Ryland ....          | 260/680 E |

|           |         |                       |           |
|-----------|---------|-----------------------|-----------|
| 3,414,631 | 12/1968 | Grasselli et al. .... | 260/680 E |
| 3,577,477 | 5/1971  | Boutry et al. ....    | 260/680 E |
| 3,607,966 | 9/1971  | Croce et al. ....     | 260/680 E |
| 3,759,840 | 9/1973  | Barker ....           | 252/432   |
| 3,764,632 | 10/1973 | Takenaka et al. ....  | 260/680 E |
| 3,778,386 | 12/1973 | Takenaka et al. ....  | 252/432   |

Primary Examiner—Paul M. Coughlan, Jr.  
Attorney, Agent, or Firm—T. H. Whaley; C. G. Ries;  
Carl G. Seutter

[57]

## ABSTRACT

Hydrocarbons such as butene may be oxidatively dehydrogenated to eg butadiene by use of a catalyst consisting essentially of oxides of molybdenum, cobalt, and boron.

6 Claims, No Drawings

OXIDATIVE DEHYDROGENATION OF  
HYDROCARBONS

## FIELD OF THE INVENTION

This invention relates to the oxidative dehydrogenation of hydrocarbons. More particularly it relates to a catalyst system particularly characterized by its ability to promote oxidative dehydrogenation. 5

## BACKGROUND OF THE INVENTION 10

As is well known to those skilled in the art, it is possible to prepare unsaturated hydrocarbons by various processes. For example, 1,3-butadiene may be prepared by dehydrogenation of n-butlenes or by the cracking of eg naphtha which yields a product stream 15 from which 1,3-butadiene may be recovered.

These processes have been continuously reviewed in order to permit attainment of reaction conditions which yield effluent streams characterized by increased yields of desired unsaturated hydrocarbon products. 20

It is an object of this invention to provide a catalyst and a process for oxidative dehydrogenation of hydrocarbons. Other objects will be apparent to those skilled in the art. 25

## STATEMENT OF THE INVENTION

In accordance with certain of its aspects, the novel process of this invention for oxidative dehydrogenation of hydrocarbons may comprise

contacting a more saturated charge hydrocarbon in vapor phase in the presence of oxygen with a catalyst consisting essentially of molybdenum oxide, cobalt oxide, and boric oxide;

maintaining said charge hydrocarbon in contact with said catalyst for 0.5-7 seconds at 350°C-550°C thereby selectively forming effluent gas containing a less saturated hydrocarbon; and

recovering said effluent gas containing said less saturated hydrocarbons. 40

## DESCRIPTION OF THE INVENTION

The more saturated charge hydrocarbon which may be treated by the process of this invention includes hydrocarbons which contain hydrogen atoms which can be removed by oxidative dehydrogenation to yield less saturated product hydrocarbons. The more saturated charge hydrocarbon may include paraffins (which may be treated by the process of this invention to yield mono-olefins) or mono-olefins (which may be treated by the process of this invention to yield di-olefins).

The preferred more saturated charge hydrocarbons may be those containing at least about 4 and preferably 4-8 carbon atoms. It is also preferred that the charge more saturated hydrocarbon be one which is in the vapor state at the conditions of operation. 55

Typical of the paraffins which may be included in the more saturated charge hydrocarbon feed may be:

n-butane  
2-methylbutane  
n-pentane  
cyclohexane  
2-ethylhexane

Typical of the mono-olefins which may be included in the more saturated charge hydrocarbon feed may be:

1-butene  
2-butene  
1-pentene  
2-pentene  
3-pentene  
2-methyl-1-pentene  
2-methyl-3-pentene  
1-hexene  
1-octene  
1-phenyl-1-butene  
cyclohexene  
2-hexene  
3-heptene

20 Preferably the more saturated charge hydrocarbon may be a mono-olefin such as a butene, more preferably 2butene.

The oxygen which may be present during the reaction may be as pure oxygen, air, oxygen-enriched air, 25 etc. Most commonly the oxygen may be provided as air.

The catalyst which may be employed in practice of the oxidative dehydrogenation process of this invention may be a composition which can be represented as consisting essentially of molybdenum oxide, cobalt oxide, and boric oxide, the mole ratio of cobalt oxide to molybdenum oxide preferably being about 1:1.

The preferred catalyst may typically be prepared by dissolving 108-180 parts (0.75-1.25 moles), preferably 35 137-151 parts (0.95-1.05 moles), say 144 parts (1.0 moles) of molybdenum oxide  $MoO_3$  in 97-338 parts (0.75-2.5 moles), say 270 parts (2.0 moles) of 28-30% aqueous ammonium hydroxide. The solution may be diluted with water to form a charge ammonium molybdate solution having a concentration of 0.2-0.3 molar, say 0.24 molar.

To the ammonium molybdate solution, there may then be added boric acid in amount of 50-125 parts (0.81-2.02 moles), preferably 75-100 parts (1.21-1.62 moles), say 90 parts (1.46 moles).

A charge cobalt nitrate solution may be prepared by dissolving 218-364 parts (0.75-1.25 moles), preferably 50 276-305 parts (0.95-1.05 moles), say 291 parts (1.0 mole) of cobalt nitrate hexahydrate  $Co(NO_3)_2 \cdot 6H_2O$  in 300-500 parts, preferably 350-450 parts, say 400 parts of water. This solution may be heated to incipient boiling typically 95°C and then added to the charge ammonium molybdate-boric acid solution, the latter also being at incipient boiling temperature, typically 95°C. 55

Upon mixing the charge ammonium molybdate solution and the charge cobalt nitrate solution, a purple precipitate is formed. This precipitate is filtered, dried at 75°C-95°C, and calcined in a stream of air at 350°C-450°C, preferably 400°C for 3-5 hours, preferably about 4 hours.

The dried precipitated oxide catalyst may, in the preferred embodiment correspond to the formula



65 wherein  $a$  is 0.75-1.25, preferably 0.95-1.05, say 1.0,  $b$  is 0.75-1.25, preferably 0.95-1.05, say 1.0, and  $c$  is 0.8-2, preferably 1.2-1.6, say c. 1.5. It will be apparent

to those skilled in the art that *a*, *b*, and *c* indicate the molar proportions of the components of the catalyst. The mole ratio of *a* to *b* may be preferably 1. Preferably, the precipitated oxide catalyst may correspond to the formula



Commonly, the dried precipitate may be ground to a particle size of 4-16 mesh, preferably about 8 mesh; and in the preferred embodiment, this catalyst may be used in the form of a gravity-packed bed.

Practice of the oxidative dehydrogenation process of this invention may be carried out by passing charge more saturated hydrocarbon, in vapor phase in the presence of oxygen, into contact with the bed of catalyst. 0.25-20 parts, preferably 0.5-5 parts, say 1 part of more saturated charge hydrocarbon and 80-99.75 parts, preferably 95-99.5 parts, say 99 parts of oxygen-containing gas may be charged. The oxygen-containing gas may be air, pure oxygen, oxygen-enriched air, etc., containing 21-100%, say 21% by weight of oxygen. The preferred oxygen-containing gas may be air. Steam may be present as diluent.

When the concentration of hydrocarbon falls within the limits of its explosive range, extra caution should be observed.

The space velocity (volume of gas per volume of catalyst per hour) VHSV may be 500-8000, preferably 1000-4000, say 2010. the corresponding time during which the gas stream is in contact with the catalyst bed may be 0.5-7 seconds, preferably 1.1-2.8 seconds, say about 1.8 seconds.

Commonly the charge may be a stream of air containing about 1% by weight of 2-butene. The charge more-saturated hydrocarbon and the oxygen may be heated to charge temperature of 350°C-550°C, preferably to at least about 400°C, say 440°C-510°C, typically to about 502°C; and the reaction is carried out at this temperature. It will be found in practice of this invention that the conversion, selectivity, and yield may decrease substantially as the reaction temperature decreases below 400°C unless the volume hourly space velocity VHSV is decreased substantially below about 4000; and accordingly a temperature of about 400°C may represent a practical preferred minimum temperature.

It may be noted that if one plots the percent conversion as a function of the value of the product of the temperature of reaction in degrees absolute and the reaction time in seconds, the attainment of conversion over 50% calls for a product value greater than about 940. This may be achieved, for example, by use of a time of 1.8 seconds and a temperature of e.g. 480°C which gives a product of 1355. Preferably, this product may be in the range of 1350-3000, and more preferably about 1350-2000. This empirical relationship may permit one to fix practical operating conditions.

During the reaction, as the gaseous mixture passes through the catalyst bed, the charge more saturated hydrocarbon is subjected to oxidative dehydration and converted to less saturated hydrocarbon. When the charge more saturated hydrocarbon is butane, the product less saturated hydrocarbon produced may be a butene. When the charge more saturated hydrocarbon is a butene, say 2-butene, in the preferred embodiment, the oxidative dehydrogenation may be found to produce 1,3-butadiene in recoverable proportions.

The content of undesirable oxygenated products (such as e.g. butyl alcohol, maleic anhydride, butyric acid, etc.,) is less than 1%; and commonly these undesired byproducts may not be found in the product in determinable quantity.

Typical effluent from oxidative dehydrogenation, e.g. of 2-butene, shows a conversion of up to 80-90%, and a selectivity of 20-40%. Commonly, the off-gas contains as the only hydrocarbons the desired e.g. 1,3-butadiene together with unconverted 2-butene (plus small quantities of 1-butene resulting from the isomerization of 2-butene); and the desired product may be readily recovered from the effluent.

#### PRACTICE OF PREFERRED EMBODIMENTS

Practice of the process of this invention may be apparent to those skilled in the art from the following examples wherein, as elsewhere in this specification, all parts are parts by weight unless otherwise stated.

#### EXAMPLE I

In this example which represents practice of the process of this invention, catalyst may be prepared (following the teaching of U.S. Pat. No. 2,691,660 q.v. also U.S. Pat. No. 2,625,519) by dissolving 144 parts (1 mole) of molybdenum oxide  $\text{MoO}_3$  in 270 parts (2 moles) of concentrated aqueous ammonium hydroxide, and then diluting the resultant solution with water to yield 4000 parts of c. 0.25 molar aqueous ammonium molybdate solution. 100 parts (1.62 moles) of boric acid  $\text{H}_3\text{BO}_3$  may then be dissolved in the solution which may then be heated to 95°C.

291 parts (1mole) of cobalt nitrate hexahydrate  $\text{Co}(\text{NO}_3)_2 \cdot 6 \text{ H}_2\text{O}$  may be dissolved in 400 parts of water and heated to 95°C. This heated solution may be poured into the molybdate-borate solution to yield a purple precipitate which is recovered by filtration, dried, and calcined in air at 400°C for 4 hours. The dried catalyst may be ground to 4-12 mesh size and placed within a 1.25-inch diameter tubular Vycor fixed bed reactor containing about 100 cc of catalyst.

A charge stream of air containing 1% of 2-butene may be heated to 416°C (780°F) and passed through the catalyst bed at space velocity VHSV of 4020 volumes/volume/hr. This corresponds to a time of reaction of about 1.25 seconds. The exit stream is passed through a water scrubber and then analyzed. The hydrocarbon portion of this stream contains 85% of 2-butene, 2% of 1-butene, 5% of 1,3-butadiene, less than 1% of other hydrocarbon constituents, and less than 1% of oxygenated hydrocarbons (e.g. maleic anhydride, butyric acid, etc.). The conversion in this example may thus be 15%; the selectivity may be 33.3%.

#### EXAMPLES II-IV

In these examples which illustrate practice of the process of this invention, the procedure of Example I is followed except that the temperature and space velocity are varied. The conditions of operation and the results are set forth in tabular form in the Table which follows the examples.

#### EXAMPLE V

In this example which represents practice of the process of this invention, catalyst is prepared (following the teaching of Bissot and Benson *Ind. Eng. Chem. Prod. Res. Dev.* 2 57-60 (1963) by dissolving 144 parts

(1 mole) of molybdenum oxide  $\text{MoO}_3$  in 130 parts of 28% aqueous ammonium hydroxide and diluting the resulting solution with 2400 parts of water to yield ammonium molybdate solution. 75 parts (1.22 moles) of boric acid  $\text{H}_3\text{BO}_3$  are dissolved in the solution which is then heated to 95°C.

A solution of 291 parts (1 mole) of cobaltous nitrate hexahydrate  $\text{Co}(\text{NO}_3)_2 \cdot 6 \text{H}_2\text{O}$  in 600 parts of water at 95°C is poured rapidly into the molybdate-borate solution yielding a purple precipitate which is filtered, dried, and calcined in air at 400°C for 4 hours. The calcined catalyst is ground to finely divided form (4-12 mesh size) and placed within a 1.25-inch diameter tubular Vycor reactor which holds a fixed bed occupying c. 100 cc.

A charge stream of air containing 1% of 2-butene is heated to 482°C (900°F) and passed through the catalyst at a space velocity VHSV of 2010 for 2 hours. The hydrocarbon portion of the exit gas stream upon analysis is found to contain 35% 2-butene, 3% 1-butene, 24% 1,3-butadiene, less than 1% of other hydrocarbon constituents, and less than 1% oxygenated hydrocarbons.

#### EXAMPLES VI-VII

Example VI represents practice of the process of this invention using the catalyst of Example V. Control Example VII, using the same catalyst, is carried out at 391°C, a temperature below the preferred minimum of 400°C.

In the Table which follows, all runs were carried out over two-hours' duration except for Examples II and VI which were carried out for one hour. The space velocity VHSV was 4020 in Examples I, II, VI, and VII, 2010 in Examples III and V, and 1005 in Example IV. All values in the Table are in mole percent except for the contact time which is in seconds, and the temperature which is in degrees Centigrade.

25

while control Example VII at 391°C and VHSV of 4020 gives no evidence of reaction. The product of the temperature (664°A) and the time (1.25 seconds) in Example VII is only 832; and attainment of desired reaction requires that this product value be raised at least to about 940. For example, if the temperature be raised to eg 415°C, the product value is 860 and the conversion would be 15%. Increasing the temperature to 482°C, raises the product value to about 947 and the conversion is about 49%.

Although this invention has been illustrated by reference to specific embodiments, it will be apparent to those skilled in the art that various changes and modifications may be made which clearly fall within the scope 10 of this invention.

I claim:

1. The method of preparing butadiene from butene which comprises

contacting said butene in vapor phase in the presence of oxygen with a catalyst consisting essentially of

$a \text{CoO} \cdot b \text{MoO}_3 \cdot c \text{B}_2\text{O}_3$

wherein  $a$  is 0.75-1.25,  $b$  is 0.75-1.25, and  $c$  is 0.8-2; maintaining said butene in contact with said catalyst for 0.5-7 seconds at 440°C-510°C thereby forming effluent gas containing butadiene; and recovering said effluent gas containing said butadiene.

2. The method of preparing butadiene as claimed in 30 claim 1 wherein said catalyst is  $\text{CoO} \cdot \text{MoO}_3 \cdot 0.8 \cdot 2 \text{B}_2\text{O}_3$ .

3. The method of preparing butadiene from butene as claimed in claim 1 wherein said charge butene is admitted to the catalyst at a volume hourly space velocity 35 VHSV of 500-8000.

4. The method of preparing butadiene from butene as claimed in claim 1 wherein said charge butene is admitted to the catalyst at a VHSV of 1000-4000.

40

TABLE

| Example | Temp. °C | Time | 2-Butene | 1-Butene | 1,3-Butadiene | Conv. | Selec. |
|---------|----------|------|----------|----------|---------------|-------|--------|
| I       | 415      | 1.25 | 85       | 2        | 5             | 15    | 33.3   |
| II      | 482      | 1.25 | 51       | 5        | 19            | 49    | 38.7   |
| III     | 502      | 2.5  | 25       | 5        | 24            | 75    | 32.0   |
| IV      | 502      | 5    | 16       | 5        | 20            | 84    | 23.8   |
| V       | 482      | 1.25 | 35       | 3        | 24            | 65    | 37.0   |
| VI      | 482      | 1.25 | 58       | 4        | 13            | 42    | 31.0   |
| VII*    | 391      | 2.5  | 100      | 0        | 0             | 0     | 0      |

\*Control

From the above table, it will be apparent that satisfactory results may be achieved in the conversion of 2-butene to 1,3-butadiene by practice of the process of this invention. Typically a conversion of up to about 84% of the charge 2-butene may be achieved with a selectivity as high as 38 + %.

It will be apparent that the reaction may be controlled to give high conversion or high selectivity; and high conversion may frequently be achieved at the expense of high selectivity.

It will also be apparent from comparison of Examples VI and VII that experimental Example VI at 482°C and VHSV of 4020 gives 42% conversion at 31% selectivity

5. The method of preparing butadiene from butene as claimed in claim 1 wherein said charge butene is contacted with said catalyst for 1.1-2.8 seconds.

6. The method of preparing butadiene from butene which comprises

contacting said butene in vapor phase in the presence of oxygen with, as catalyst,  $\text{CoO} \cdot \text{MoO}_3 \cdot 0.8 \text{B}_2\text{O}_3$ ; maintaining said butene in contact with said catalyst for 1.1-2.8 seconds at 440°C-510°C thereby forming effluent gas containing butadiene; and recovering said effluent gas containing said butadiene.

\* \* \* \* \*